

## UNITED STATES PATENT OFFICE

2,153,963

MANUFACTURE OF ELASTIC PRODUCTS  
WITH A TEXTILE BASIS

Léon Sylvain Max Lejeune, Paris, and Emile Jean Albert Lejeune, Lille, France, assignors, by mesne assignments, to Hevaloid Corporation, Dover, Del., a corporation of Delaware

No Drawing. Application September 2, 1936, Serial No. 99,149. In France April 5, 1933

22 Claims.

(Cl. 28—1)

Our present application has for its object the manufacture of new elastic products with a textile basis and is a continuation-in-part application of our prior application, Serial No. 690,760, filed September 23, 1933.

The invention relates more particularly to the manufacture of elastic textile fabrics, that is to say, products of every variety that have a textile basis, impregnated or associated with an elastic or plastic substance such as rubber. The invention comprises the improved elastic fabrics themselves and also the herein described process of making the same. Its main object is to obtain fabrics (including the linear elements whereof they are composed) which possess the qualities of strength and elasticity in a very high degree, together with relatively high transverse compressibility, and to obtain such products by a process which is even more economical than the processes whereby the highest grades of elastic textile fabrics are now produced. The elastic textile products obtained by the process herein described, and which are included within the present invention, are characterized and distinguished from other commercial products of the same class chiefly by the following characteristics: first, a relatively high degree of tensile strength; second, a relatively high degree of residual elasticity, that is to say, of elasticity which remains after the properties of the fabric have been permanently fixed; third, a physical union of the basic textile fabric and the rubber which is so close and tenacious as to amount to virtual homogeneity, this being a very distinctive and conspicuous characteristic of the new products; fourth, a relatively high degree of transverse compressibility; fifth, a thorough impregnation with rubber or the like which can be made to penetrate to all parts of the fibrous mass.

The invention specially contemplates the employment of cotton fibers, but can be successfully applied to other textiles, such as jute, flax, hemp, ramie, etc. It is to be understood that where "rubber" is mentioned herein, other elastic or plastic substances suitable for the purposes of the invention are included within the meaning of the word.

The process whereby fabrics and linear elements having the above and other desirable properties are obtained according to the invention is

characterized mainly by the initial step or operation, according to which the primary fibrous elements (rovings) constituting the textile base are subjected to what is herein termed an "inverse twist", whereby said rovings are formed into elements having novel and distinctive characteristics. The ultimate fabric or product is made of these linear elements. Said linear elements may be formed of commercial rovings of any of the grades (or degrees of initial twist) that are readily obtainable. The first step in the "inverse twist" operation is to take two (or more) rovings and impart to each individually such a super-twist (in the same direction as its primary twist) that they can no more readily be drawn out substantially, for example, in the case of rovings of size, 2.5 (French nomenclature) until the total twist aggregates, say, 200 turns per meter, more or less. Obviously, if rovings are obtainable which have already been given a sufficiently high degree of twist, which varies within somewhat wide limits according to the ultimate product sought and to other variable conditions, the specified over-twist will not be required. Two or more such fibrous units, each twisted in the same direction and to the predetermined degree, are brought together and are twisted as an assembly in the opposite direction to that in which the individual rovings were twisted. The best result is obtained when this reverse twist approximates the same number of turns as the total initial twist imparted to the individual units of the linear elements; for then the textile elements will be found to be in a state of approximate equilibrium, that is, a state wherein the element has little or no tendency to untwist.

As has already been stated, the amount of twist given to the individual rovings in the first instance and then given to the assembled rovings in the reverse direction depends upon several variable conditions, but it is easy to ascertain in each particular case what amount of twist, that is, the number of turns per linear unit, should be given in each direction. It has been found that particularly good results are obtained with linear elements each composed of two cotton rovings of size No. 2.5, and to which a total twist of 200 turns per meter in each direction has been given. If, for example, the initial ordinary twisting of the roving was 80 turns, a supplemental twisting

of 120 turns would be required to make the desired total. As is known, when a cotton roving of size No. 2.5 has been given a twist of approximately 200 turns per meter, it cannot be substantially drawn out. Therefore, it suffices, in order to give a sufficiently definite idea of the amount of twist that should be imparted to the rovings, to state that the advantages of the invention will be realized in a satisfactory degree when the rovings are twisted, before being assembled, to such an extent that they cannot be substantially drawn out. A linear element so made is found to possess, contrary to what would be expected, a higher degree of tensile strength than the sum of the tensile strength of the several units. Such a linear element, when treated according to this invention as will be explained hereafter, is found to possess extraordinary degrees both of strength and elasticity. And when it is impregnated with rubber or the like, the resulting elastic products approach much closer than any now obtainable the ideals set forth above.

The linear elements themselves (the direct products of the inverse twist) are specially characterized by structural uniformity as regards the arrangement of the fibers composing each of the fibrous units relatively to each other, in consequence of which each unit is in a state of approximately uniform openness throughout and hence is readily permeated even to the center by the swelling agent. Moreover, this structural openness remains after the treatment according to the invention, so that the element is readily permeable even to the center by the elastic substance in solution or suspension. During the imparting of the reverse twist to the assembly of supertwisted rovings each unit undergoes a compound movement: first, there is the movement whereby the several units are twisted into an inversely twisted element, in the course of which they rotate on a common axis, each unit revolving around the other; second, there is the movement whereby the fibrils of each unit are rotated with reference to each other in a direction opposite to the twist initially imparted to them, the result being a rearrangement of the constituent fibrils relatively to each other and also a substantial relaxation of the strong centripetal compression exerted by the outer fibrous helices of the unit resulting from the initial twist. Thus is brought about a unique structural condition of the textile linear element as a whole, which condition is conducive to the most favourable results from the successive steps of treatment and impregnation.

The treatment to which are subjected the textile elements according to the invention essentially consists in a treatment without tension by means of a contracting and swelling agent such as caustic soda lye, in conditions such that the linear element have their fibres strongly contracted and swollen without however being subjected to substantial mutual compression.

In contrast with what has been heretofore effected when textile fabrics or elements have been treated with hydrolyzing agents (in which case the elasticity of the product is merely that of the fiber proper and the tensile strength is that of the impregnating material) the process of the present invention effects a re-arrangement of the swollen and contracted fibers such as to form a very open texture, while there is nevertheless a certain twisting, or a particular path of individual fibers which is equivalent to a twist, with a consequent bonding together and inter-

locking of the fibers without diminution of the elasticity, but on the contrary with an enhancement both of the elasticity and also of the tensile strength of the textile base. In consequence of the rearrangement of the individual fibers with respect to each other and of the contracting and swelling effect resulting from the action of the soda lye or the like, and also of the additional elasticity imparted by the impregnating substance, the elasticity of the linear elements themselves and therefore that of webs or fabrics composed thereof, is much greater than that of the fiber itself or of a thread which has not been subjected to the described inverse twist and the subsequent swelling and contracting treatment.

The particular agent whereby the contraction and distention of the inversely twisted linear elements is to be effected will be selected according to the particular product in view, preference being given to agents, acid or alkaline as the case may be, that will produce a maximum, and as nearly as possible, a homogeneous swelling and shortening effect; and to agents that do not cause deterioration of the fiber. Agents which transform the fiber without deterioration into hydrocellulose may be used with advantage. The best results thus far have been obtained with vegetable fibers by the use of alkalis, especially soda, under proper conditions of concentration, temperature, and duration of treatment.

This treatment yields a swollen and contracted linear element in which the fibers are not appreciably compressed one against the other. However, the reciprocal interlocking of the fibers is sufficiently increased by the treatment to add substantially to the tensile strength of the element. The elasticity also is considerably increased, not only by reason of the transformation of the substance of the fiber into one that is more elastic, but also by reason of the condition into which the linear element as a whole has been brought. Furthermore, the residual elasticity of an inversely twisted linear element so treated, that is to say, the elasticity which exists after a tension produced by a force exceeding that which produces the first permanent elongation, is greatly augmented.

In carrying out the contracting and swelling treatment according to the invention, it may be useful to employ a wetting agent, in order that the textile elements be fully wetted by the bath in which they are immersed. As wetting agent there may be employed any wetting agent which is commonly known for the usual treatments of textiles with liquids.

The textile elements or textile products are allowed to remain in the bath under conditions such as will be more fully described in relation with the examples given hereafter; afterwards the textile is extracted from the bath and is expressed so that the greatest part of the bath may be recovered.

The steps of the process which follow the inverse twist operation may be performed in either of several different sequences. It might seem that the logical order of procedure in making an elastic fabric would be to subject the inversely twisted linear element first to the action of the contracting and swelling agent and then to impregnation with the selected elastic or plastic substance, and then (either before or after vulcanization) to weave said element into a fabric; and this order of procedure may be adopted with satisfactory results. Preferably, however, the

Linear elements formed by the described inverse twist are woven into fabric and afterwards treated with the contracting and swelling agent and finally impregnated with rubber or the like and vulcanized, if desired. This order of procedure is preferred partly because the products thereby obtained are found to be superior, in respect to tensile strength and residual elasticity, to those obtained by the order of procedure first stated above; and also because thereby a substantial saving is effected in the cost of operation; the principal reasons being that there is great difficulty in weaving the rubberized elements and that when the linear elements are treated and impregnated before being woven into fabric, it is necessary to subject the fabric to further impregnation.

According to another modification, the linear textile elements formed by the described inverse twist may be treated with the contracting agent, then be woven into a fabric, and then be impregnated with an elastic or plastic material.

In the fabrication of elastic textile products that are not woven into fabrics, the inversely twisted linear elements after treatment with the contracting and swelling agent and impregnation with rubber or the like, may be formed into the desired product by any appropriate means, as by the twisting of a plurality of such elements into a cord or rope, and eventually re-impregnating the so formed product.

Although the chemical agents used in the process of this invention are or may be of the same nature (alkalis) as those employed in the process known as "mercerizing", it is of interest to note that the contraction and swelling step of this invention is not the same as the one encountered in common mercerization and its results are essentially different. For instance, in the common operation of mercerizing the initial linear dimensions are not altered; in other words, there is no contraction, a tension being exerted at a given period. According to the present invention there is no tension on the textile fabric or elements during the soda lye treatment, but on the contrary, the textile fabric or element is permitted freely to contract. Moreover, the swelling and contracting agent permeates and acts, preferably upon every part of the fibrous mass, under conditions of concentration, temperature, and duration of treatment which differ from those of mercerization. The textile fabrics or elements do not have, after the swelling and contraction treatment of the present invention, the silk-like lustre that characterizes mercerized products; but on the contrary, when examined under a microscope, they are seen to have a wrinkled and rugged surface.

The described treatment with soda lye and washing has the effect of increasing substantially the tensile strength of the linear elements and hence that of the fabric composed thereof. The structure is perceptibly different under a magnifying glass, particularly in that the element remains in an open and permeable condition, and also in that there are few detached fibers, nearly all being aggregated and consolidated together and hence contributing to the strength of the element.

Preferably, after having been subjected to the treatment with the bath of contracting and swelling agent, the textile products according to the invention are subjected to a boiling treatment, which is carried out under the conditions usual

for such a treatment in the textile industry, for example with the aid of carbonate of soda lye, at the high temperature convenient for boiling.

After this boiling treatment, the textile products preferably are washed with warm water, then with cold water, and afterwards they are submitted to a treatment with hydrochloric acid or the like, then are washed and finally are carefully dried. The textile product thus obtained is ready for impregnation.

We will now describe more in detail and by means of illustrative and non-limiting examples, how the process of this invention may be carried out with practical success and so as to accomplish the best results in view of obtaining highly impregnable textile products ready for impregnation to the core.

#### *Formation of inversely twisted linear element*

An ordinary cotton roving, for example a roving of size 2.5, possessing no appreciable tensile strength, is given a total twist of say 200 turns per meter to the right. A second roving of the same sort is twisted in the same direction and to the same degree. These two super-twisted rovings are brought together, as by means of an ordinary twisting machine and are twisted 200 turns per meter to the left about an hypothetical medial axis common to the two rovings. This inverse twist causes a swelling of the linear element, while at the same time it eliminates or almost completely relaxes the reciprocal compression exerted by the constituent fibers between themselves.

#### *Treatment with caustic soda*

*First example.*—An inversely twisted linear element, formed as just described, is soaked in caustic soda lye of a concentration of 5-35° Bé. at a temperature of 8-18° C. for a suitable time to effect the above described transformation, which time may vary from 5 to 30 minutes, according to the degree of swelling and contraction desired. With a caustic soda lye of 35° Bé. at a temperature of 18° C. to which has been added, in the commonly used proportions, a suitable wetting agent and with a treatment of thirty minutes duration, a pronounced swelling and contraction effect, reaching 30%, is obtained.

A thread of this kind weighing, after treatment with soda under the above conditions, 500 mg. per meter attained a tensile strength of 9.5 kg. with an elongation of 30% while a cord of cotton of the same weight broke at 7.5 kg. with an elongation of only 25%.

The new product shows a very great transverse compressibility and, as will be explained in detail later, a great capacity for penetration by elastic or plastic materials.

*Second example.*—Two inversely twisted linear elements, formed by the same process as just described of two rovings of superior Egyptian cotton of 32-33 mm. length of fiber, carded quality 2.5, French nomenclature (2500 m. to 500 grams), were each treated according to the process of this invention, but under somewhat different conditions respectively. The conditions and results of the respective treatments are given in Tables I and II below. Table III gives the results of tests for tensile strength and elongation at breaking point of the linear element in the raw state, as scalded, and as both scalded and bleached.

TABLE I  
Concentration: 30° Bé.; temp. 18° C.; duration 15 minutes

|       | Raw                     |                              | Scalded                 |                              |
|-------|-------------------------|------------------------------|-------------------------|------------------------------|
|       | Tensile strength in kg. | Elongation at breaking point | Tensile strength in kg. | Elongation at breaking point |
| 7.350 | Percent 23.76           | 8.500                        | Percent 26.00           |                              |
| 7.250 | 22.75                   | 8.400                        | 25.75                   |                              |
| 7.700 | 25.00                   | 8.950                        | 28.50                   |                              |
| 7.300 | 25.00                   | 8.950                        | 26.50                   |                              |
| 7.400 | 23.00                   | 8.300                        | 27.00                   |                              |
| Mean  | Mean                    | Mean                         | Mean                    |                              |
| 7.420 | 23.9                    | 8.680                        | 26.75                   |                              |

Weight 520 grams per 1,000 meters, fibers not tensioned.

TABLE II  
Concentration: 20° Bé.; temp. 8° C.; duration 30 minutes

|       | Raw                     |                              | Scalded                 |                              |
|-------|-------------------------|------------------------------|-------------------------|------------------------------|
|       | Tensile strength in kg. | Elongation at breaking point | Tensile strength in kg. | Elongation at breaking point |
| 7.600 | Percent 22.0            | 8.600                        | Percent 31.00           |                              |
| 7.650 | 23.0                    | 8.750                        | 29.00                   |                              |
| 7.500 | 23.5                    | 8.300                        | 28.75                   |                              |
| 7.600 | 23.5                    | 8.300                        | 29.75                   |                              |
| 7.650 | 23.0                    | 8.700                        | 28.00                   |                              |
| Mean  | Mean                    | Mean                         | Mean                    |                              |
| 7.600 | 23                      | 8.560                        | 29.3                    |                              |

Weight 520 grams per 1,000 meters, fibers not tensioned.

TABLE III  
Before treatment with soda

|   | Raw                     |                              | Scalded                 |                              |
|---|-------------------------|------------------------------|-------------------------|------------------------------|
|   | Tensile strength in kg. | Elongation at breaking point | Tensile strength in kg. | Elongation at breaking point |
| 5 | Percent 9               | 5.600                        | Percent 10.8            |                              |

Third example.—Taking two rovings of cotton of total weight 380 mg. per meter; twisting them 140 turns per meter to the right, then, after assembly, 140 turns to the left, and treating them as stated above, a thread weighing 500 grams per 1000 meters is obtained, the longitudinal contraction in the treatment having been 30%, while the initial tensile strength of the original thread, twisted 140 turns, was 6.2 kg. and the elasticity 10%. This treated element has a tensile strength of 9.5 kg. and an elasticity of 36%.

In comparison, an ordinary cord of the same material, also weighing 500 grams per 1000 meters, comprising an assembly of fifteen No. 18 threads, a spinning twist of 800 turns, a twisting torsion of 690 turns in the same direction, and a cording twist of 350 turns, was found to possess the following characteristics: Tensile strength—7.500 kgs.; elongation at breaking point—24%; threads very tightly squeezed together.

With jute, treated as described above, an elas-

ticity of 25% was obtained; whereas this fiber, as is well known, has only 3% elasticity in its natural state and is in consequence very brittle.

With respect to the treatment which is carried out subsequently to the contracting and swelling treatment just above described, as before said, the textile fabric—assuming that linear elements woven into a fabric are contemplated—remains in the bath during the time above indicated. Afterwards the fabric is extracted from the bath and expressed so as to recover as much as possible of the said bath.

The fabric is then carefully washed, and then submitted to the treatment of boiling. Said boiling is performed under the ordinary conditions of such well-known operation, i. e. by means of a lye of carbonate of soda of 3%, to which there is added a soda soap of 1.5% under a pressure of 1.5 atm. corresponding to a temperature of 113° C. for 4 hours. The percentage always is calculated with respect to the weight of dry cotton.

After having been boiled, the fabric is washed with warm water at 90° for about 1 hour, carefully washed with cold water, neutralized through a solution of trade hydrochloric acid of 0.5 Bé., then again washed till the chlorides are eliminated. Finally the treated fabric is carefully dried so that there only remains about 7% of wetness with respect to the weight of the dry cotton. The fabric is then ready for impregnation.

Instead of making with the so called "inverse twists" a fabric which is subjected to a swelling and contacting operation by means of a swelling and contracting agent, such as soda lye according to the hereabove described process, further subjecting the said fabric to a boiling treatment such as a treatment by a diluted soda carbonate lye under pressure at an increased temperature during several hours, the fabric being then washed, eventually dried and impregnated with elastic or plastic material, the inverse twists may be first subjected to the aforesaid swelling and contracting treatment, then woven in the form of a more or less closed mesh fabric and the so formed fabric is then subjected to a boiling treatment such as the above mentioned boiling treatment, then washed, eventually dried and impregnated with elastic or plastic material.

The linear elements or fabrics, previously treated as described, may be made to take up an amount of rubber equal in weight to or more than that of the fabric itself by simple impregnation without repetition.

#### Impregnation with elastic or plastic substance

The effect of the inverse twist and the swelling and contracting treatment is to bring the textile fabric or element as a whole and its component fibers individually into a condition that is very favorable to complete and thorough impregnation with rubber or other elastic or plastic substance; insomuch that the desired result can be obtained without the aid of costly vacuum and pressure appliances and operations such as have been heretofore used to complete penetration of the fibrous mass by the rubber or like material.

An important object of the impregnation operation is to fix permanently the properties of strength and elasticity that have been imparted to the fabrics or linear elements by the operations of inverse twisting and of swelling and contraction.

For the purpose of the impregnation operation, use may be made of a natural or synthetic sus-

pension or dispersion of rubber or other elastic or plastic material (balata, etc.), or of a solution of one or other of those substances.

The impregnating liquid may be applied by means of brushes or in a calendering machine, or preferably by soaking. Vacuum or pressure, or both, may if desired be used in special cases to aid the impregnation; but, as already stated, those aids are not needed in order to obtain the benefits of the invention.

When a solution is used for the impregnation, it is necessary, of course, to dry the element previously; but when latex or analogous natural or artificial suspension is used, drying is not necessary.

Preferably the impregnation is carried out by immersion of the textile product in a bath of latex, containing for example 40% of dry rubber together with the vulcanising products. The impregnation occurs, preferably without vacuum or pressure being applied, in vats or other receptacles which are closed with a cover which is sufficiently tight to prevent the ammonia from evaporating, which latter would result in a coagulation of the surface of the bath. After each impregnating operation, the ammonia content of the bath is brought to the required degree by adding thereto a solution of trade ammonia.

The degree of impregnation desired will determine the duration of the treatment. Latex, natural or concentrated and preferably containing all elements necessary for vulcanization, is specially suitable.

After the impregnation, the fabric or other textile product is placed in conditions suitable for coagulating of the rubber. To effect this, the ammonia is allowed to evaporate or is neutralized.

When the coagulation is effected, the impregnated textile product, e. g. fabric, is placed in such conditions that the water still contained therein evaporates for the greater part. To effect this, the fabric or the like can be calendered with an usual calender so as to remove the greatest possible part of water, afterwards the product is dried in any suitable manner. Care shall be taken that the temperature of the drying apparatus be lowered as the fabric dries.

The quantity of water remaining at that time in the textile fabric or product will not exceed 4% of the weight of the impregnated fabric.

In most cases, the impregnating treatment of the final impregnated products to be obtained is followed by a vulcanization. The fabric when impregnated are preserved until it is desired to vulcanize the same. For this purpose they are kept preferably in warehouses which are dimly lighted and not too moist. When it is desired to obtain fabrics composed of several plies or thicknesses, the component plies are to be stuck together prior to warehousing in order to prevent oxidation of the surfaces of the plies.

The impregnated inverse twisted linear elements or fabrics made therefrom may be stretched (before or after drying but in all cases before vulcanization) for the purpose of diminishing their residual elasticity, which stretching in the case of woven fabrics may be either in one direction only or in both.

The drying or vulcanization will fix the initial elongation so determined, which will serve as a starting point for further elongation whereby the ultimate residual elasticity will be determined. By this procedure not only may the elasticity of a web be entirely eliminated in a direction in

which it is not desired (as in the transverse direction of a belt) but also thereby surface area that has been lost through shrinkage may be regained. In the case of a very elastic fabric the initial length (or width) may be exceeded and the dimension thus attained may be fixed.

The product is vulcanized preferably under a pressure of about 25/30 kg. per cm<sup>2</sup>.

The invention also comprises means for preventing any substantial bulging or warping of the fabric due to the fact that the selvages of the same are always more compressed than the rest of the fabric. In order to avoid any risk of such bulging, it is preferred, before the operation of stretching and vulcanization, to cut the selvages of the fabric in such a manner that the strips or sheets finally obtained are prevented from bulging. As aforesaid, the removal of the selvages by cutting should take place before the fabric is stretched.

In the tables below are given the practical results of the impregnation by rubber latex of linear elements corresponding to those of Tables I and II above. The rubberizing was effected by immersion in natural latex for four hours, followed by a coagulation with acetic acid, drying and vulcanization.

*Impregnation of elements treated as per Table I,  
supra*

| Raw                     |                                                      | Scalded                                   |                                                      |
|-------------------------|------------------------------------------------------|-------------------------------------------|------------------------------------------------------|
| Tensile strength in kg. | Elongation at breaking point                         | Tensile strength in kg.                   | Elongation at breaking point                         |
| 8.700                   | Percent<br>20.00<br>20.50<br>21.00<br>20.00<br>20.00 | 9.350<br>8.700<br>8.750<br>8.650<br>9.000 | Percent<br>22.00<br>22.00<br>22.50<br>21.00<br>21.50 |
| Mean                    | Mean                                                 | Mean                                      | Mean                                                 |
| 8.700                   | 20.3                                                 | 8.900                                     | 21.8                                                 |

*Impregnation of elements treated as per Table II,  
supra*

| Raw                     |                                                      | Scalded                                   |                                                      |
|-------------------------|------------------------------------------------------|-------------------------------------------|------------------------------------------------------|
| Tensile strength in kg. | Elongation at breaking point                         | Tensile strength in kg.                   | Elongation at breaking point                         |
| 8.950                   | Percent<br>19.50<br>18.00<br>18.25<br>18.50<br>19.00 | 9.100<br>8.350<br>9.200<br>8.900<br>8.650 | Percent<br>19.75<br>19.00<br>19.00<br>19.00<br>19.00 |
| Mean                    | Mean                                                 | Mean                                      | Mean                                                 |
| 8.730                   | 18.65                                                | 8.840                                     | 18.15                                                |

The above tables show that, starting with an inversely twisted linear element weighing 520 grams per 1000 meters and having a tensile strength of 7.5 kilograms to 9 kilograms, with an elongation at breaking point of 24-30%, and impregnating it with rubber latex to 18% of its initial weight, one obtains a rubberized textile thread having a tensile strength of 9 kilograms, with an elongation of 20-23% and a residual longitudinal elasticity which varies from 5% to 5.5% under a tension of 4.5 kilograms. This

residual longitudinal elasticity is superior by 20% to that of the non-impregnated twist.

Thus it will be noted that the tensile strength and the elongation (especially the latter) of such an impregnated inverse twist are considerably higher than those of an impregnated cord, for the same weight of the same textile material and the same impregnating substance. These differences arise from the fact that, owing to the structure of the ordinary cords they can be only superficially impregnated, from which it results that the fibers of those cords are subject to varying operating conditions, according to whether or not they are in the outer zone which is reached by the impregnating liquid. In the impregnated textiles of the present invention, on the contrary, the elongation is not produced by the sliding of the fibers relatively to each other, but by the stretching of the fibers themselves. On the other hand, because of the peculiar arrangement of the fibers relatively to one another and the absence of compression, the straightening of the fibers is less hindered than in an ordinary impregnated cord. Moreover, the homogeneity of the product of the present invention is such that all the fibers undergo stress or strain simultaneously to approximately the same extent. The increase of strength is due largely to this cause.

The products of the above described process can be readily distinguished by their observable characteristics and properties from products of the same class hitherto known. The inversely twisted linear element itself, which is an intermediate product, has distinctive characteristics whereby it can be identified. It imparts those distinctive characteristics to the final products of which it forms the textile basis. Said linear element is specially characterized in that while the textile units composing it are twisted together, they are individually in such condition of openness that the constituent fibers lie close together without reciprocal compression, there being practically no centripetal pressure exerted by the fibers upon others nearer the center, and practically no reciprocal pressure exerted by the rovings upon each other. Consequently the linear element as a whole is in a state of approximately uniform openness to penetration by the swelling and contracting agent and by the rubber dispersion or solution. Penetration by the rubber is promoted also by the structure of the outer and inner surfaces of the fibers themselves. The fibers of the element are also, as the result of the inverse twist, found in the form of helices and in such a condition that when a tensile longitudinal stress is exerted upon the element the fibers are all straightened substantially to the same extent and are tightened together and are all subjected to the same stress. This peculiar structural condition, which is readily observable under a magnifying glass of moderate power, is the principal cause of the valuable properties, already described, of the final products of this invention—such as their great tensile strength, their high coefficient of residual elasticity, and of transversal compressibility, the large proportion of rubber incorporated in the textile, and the remarkably tenacious cohesion of the rubber and the fibers. This cohesion is such as to integrate the two constituents, forming what is, for all practical purposes, a homogeneous product.

It is to be understood that the fabrics made according to the present invention comprise all

kinds of woven fabrics, knitted fabrics or cord fabrics and that they can be used for manufacturing all products or articles in which impregnated textiles are used.

What we claim is:

1. Process for the manufacture of elastic textile products, which comprises twisting each of a plurality of rovings in the same direction, bringing together the twisted units, twisting the assembled units in the direction opposite to that in which the individual units were twisted until an appreciably opened linear element is obtained, and treating without substantial tension the linear element so formed with a contracting and swelling agent. 5

2. Process for the manufacture of elastic textile products, which comprises twisting each of a plurality of rovings in the same direction, bringing together the twisted rovings, twisting the assembled units in the direction opposite to that in which the individual units were twisted until an appreciably opened linear element is obtained, weaving a number of linear elements so formed into a fabric, and treating the fabric without substantial tension with a contracting and swelling agent. 10

3. Process for the manufacture of elastic textile products, which comprises twisting each of a plurality of rovings in the same direction, bringing together the twisted rovings, twisting the assembled units in the direction opposite to that in which the individual units were twisted until an appreciably opened linear element is obtained, weaving a number of linear elements so formed into a fabric, treating the fabric without substantial tension with a contracting and swelling agent, and impregnating the fabric with rubber. 15

4. In the process of claim 3, the removal of a part of the elasticity of the linear element by tension and fixing the degree of elasticity thus attained by vulcanisation. 20

5. Process for the manufacture of elastic textile products, which comprises twisting each of a plurality of rovings in the same direction, bringing together the twisted units, twisting the assembled units in the direction opposite to that in which the individual units were twisted until the number of turns of the reverse twist equals approximately that of the previous twist of the individual units, and treating without substantial tension the linear element so formed with a contracting and swelling agent. 25

6. Process for the manufacture of elastic textile products, which comprises twisting each of a plurality of rovings in the same direction, bringing together the twisted rovings, twisting the assembled units in the direction opposite to that in which the individual units were twisted until the number of turns of the reverse twist equals approximately that of the previous twist of the individual units, weaving a number of linear elements so formed into a fabric, and treating the fabric without substantial tension with a contracting and swelling agent. 30

7. Process for the manufacture of elastic textile products, which comprises twisting each of a plurality of rovings in the same direction, bringing together the twisted rovings, twisting the assembled units in the direction opposite to that in which the individual units were twisted until the number of turns of the reverse twist equals approximately that of the previous twist of the individual units, weaving a number of linear elements so formed into a fabric, treating the fabric without substantial tension with a con- 35

- tracting and swelling agent, and impregnating the fabric with rubber.
8. An elastic product having a textile basis formed of linear elements each comprising a plurality of rovings which have been twisted individually in the same direction and aggregately in the opposite direction and of rubber uniformly distributed throughout the fibrous mass and firmly united to the individual fibers.
- 10 9. An elastic product having a textile basis composed of linear elements, each comprising a plurality of supertwisted rovings firmly twisted together in the direction opposite to that of the twist of the said rovings, the individual units being in a state of uniform openness to penetration by liquids and of absence of internal compression, the constituent fibers being an assemblage of helices having approximately the same pitch.
- 20 10. A woven fabric formed of linear textile elements comprising each a plurality of supertwisted rovings twisted together in the direction opposite to that of the twist of the said rovings, the individual units being in a state of uniform openness to penetration by liquids and without reciprocal compression between the constituent fibers, said elements being impregnated with an elastic substance which fills the interstices between them and binds the fibers into a dense and strongly coherent fabric.
- 30 11. A linear textile element comprising a plurality of rovings which have been twisted individually in the same direction and are twisted together in the opposite direction, the individual rovings of the assembly being in a state of uniform openness to penetration by liquids and without reciprocal compression between the constituent fibers, said fibers being contracted and swollen.
- 40 12. Process for the manufacture of elastic textile products, which comprises twisting each of a plurality of rovings in the same direction, bringing together the twisted units, twisting the assembled units in the direction opposite to that in which the individual units were twisted until an appreciably opened linear element is obtained, and treating without substantial tension the linear element so formed with a contracting and swelling agent added with a wetting agent, subjecting then the linear element to a boiling treatment, to washing and drying.
- 50 13. Process for the manufacture of elastic textile products, which comprises twisting each of a plurality of rovings in the same direction, bringing together the twisted rovings, twisting the assembled units in the direction opposite to that in which the individual units were twisted until an appreciably opened linear element is obtained, weaving a number of linear elements so formed into a fabric and treating the fabric without substantial tension with a bath formed of a contracting and swelling agent and added with a wetting agent, subjecting then the fabric to a boiling treatment and then to washing and dry-  
ing.
- 60 14. Process for the manufacture of elastic textile products, which comprises twisting each of a plurality of rovings in the same direction, bringing together the twisted rovings, twisting the assembled units in the direction opposite to that in which the individual units were twisted until an appreciably opened linear element is obtained weaving a number of linear elements so formed into a fabric, treating the fabric without substantial tension with a contracting and swelling agent
- 70 added with a wetting agent, subjecting then the fabric to a treatment of boiling, then to washing and drying, and impregnating the treated fabric with elastic material.
15. Process for the manufacture of elastic textile products, which comprises twisting each of a plurality of rovings in the same direction, bringing together the twisted rovings, twisting the assembled units in the direction opposite to that in which the individual units were twisted until an appreciably opened linear element is obtained, weaving a number of linear elements so formed into a fabric, treating the fabric without substantial tension with a contracting and swelling agent added with a wetting agent, subjecting then the fabric to a treatment of boiling, then to washing and drying, impregnating the treated fabric with elastic material, allowing the same to coagulate and then to dry, stretching the linear elements to remove part of the elasticity thereof and fixing the degree of elasticity thus attained by vulcanization.
16. Process for the manufacture of elastic textile products, which comprises twisting each of a plurality of rovings in the same direction, bringing together the twisted units, twisting the assembled units in the direction opposite to that in which the individual units were twisted until the number of turns of the reverse twist equals approximately that of the previous twist of the individual units, treating without substantial tension the linear elements so formed with a contracting and swelling agent added with a wetting agent, subjecting then the linear elements to a boiling treatment, then to washing and drying.
17. Process for the manufacture of elastic textile products, which comprises twisting each of a plurality of rovings in the same direction, bringing together the twisted rovings, twisting the assembled units in the direction opposite to that in which the individual units were twisted until the number of turns of the reverse twist equals approximately that of the previous twist of the individual units, weaving a number of linear elements so formed into a fabric, treating the fabric without substantial tension with a bath formed of a contracting and swelling agent and added with a wetting agent, subjecting then the fabric to a treatment of boiling and then to washing and drying.
18. Process for the manufacture of elastic textile products, which comprises twisting each of a plurality of rovings in the same direction, bringing together the twisted rovings, twisting the assembled units in the direction opposite to that in which the individual units were twisted until the number of turns of the reverse twist equals approximately that of the previous twist of the individual units, weaving a number of linear elements so formed into a fabric, treating the fabric without substantial tension with a contracting and swelling agent added with a wetting agent, subjecting then the fabric to a boiling treatment, then to washing and drying and impregnating the fabric with an elastic material.
19. Process for the manufacture of elastic textile products, which comprises twisting each of a plurality of rovings in the same direction, bringing together the twisted rovings, twisting the assembled units in the direction opposite to that in which the individual units were twisted until the number of turns of the reverse twist equals approximately that of the previous twist of the individual units, weaving a number of linear elements so formed into a fabric, treating the fabric

without substantial tension with a contracting and swelling agent added with a wetting agent, subjecting then the fabric to a boiling treatment, then to washing and drying, impregnating the fabric with an elastic material, coagulating the same and drying it, cutting the selvages of the fabric and subjecting the said fabric to stretching and vulcanization.

5 20. A linear textile element comprising two rovings of French size No. 2.5 which have been 10 twisted individually in the same direction for about 200 turns and are twisted together in the opposite direction also for about 200 turns the two individual rovings of the assembly being in a state 15 of uniform openness to penetration by liquids and without reciprocal compression between the constituent fibers, said fibers being contracted and swollen as well as boiled.

21. A woven fabric formed of linear textile elements comprising each two rovings of French 20

size No. 2.5 supertwisted up to about 200 turns and twisted together in the direction opposite to that of the twist of the said rovings also for about 200 turns, the two individual units being in a state of uniform openness to penetration by 5 liquids and without reciprocal compression between the constituent fibers, said elements being impregnated with an elastic substance which fills the interstices between them and binds the fibers into a dense and strongly coherent fabric.

22. An elastic product having a textile basis formed of linear elements each comprising two rovings of French size No. 2.5 which have been 10 twisted individually in the same direction for about 200 turns and aggregate in the opposite 15 direction also for about 200 turns and of rubber uniformly distributed throughout the fibrous mass and firmly united to the individual fibers.

LÉON SYLVAIN MAX LEJEUNE.

EMILE JEAN ALBERT LEJEUNE.

20